

G. F. DOWNS.

PROCESS FOR COATING MOLDS FOR METAL INGOTS.

APPLICATION FILED DEC. 16, 1916.

1,243,717.

Patented Oct. 23, 1917.

2 SHEETS—SHEET 1.



1,243,717.

G. F. DOWNS.

PROCESS FOR COATING MOLDS FOR METAL INGOTS.

APPLICATION FILED DEC. 16, 1916.

Patented Oct. 23, 1917.

2 SHEETS—SHEET 2.



Witnesses:

J. H. Alfreds  
D. Darbenque

Inventor:  
George F. Downs  
by James McElroy Atlys

# UNITED STATES PATENT OFFICE.

GEORGE FRANCIS DOWNS, OF BUFFALO, NEW YORK.

## PROCESS FOR COATING MOLDS FOR METAL INGOTS.

1,243,717.

Specification of Letters Patent.

Patented Oct. 23, 1917.

Application filed December 16, 1916. Serial No. 137,417.

*To all whom it may concern:*

Be it known that I, GEORGE F. DOWNS, a citizen of the United States, and a resident of Buffalo, in the county of Erie and State 5 of New York, have invented certain new and useful Improvements in Processes for Coating Molds for Metal Ingots; and I do hereby declare that the following is a full, clear, and exact description thereof, reference being had to the accompanying drawings, and to the letters of reference marked thereon, which form a part of this specification.

This invention relates to an improved 15 process for coating the inside surface of steel-ingot-casting molds, and consists of the matters hereinafter described and more particularly pointed out in the appended claims.

20 A factor of primary importance in steel making is the preparation of the steel ingot itself, and particularly as to the formation and condition of its outer surface. After the molten metal has been poured into the mold and when it is being allowed to cool, it is of prime necessity that the outer surface of the ingot shall not stick to the mold during the time it is cooling. During this stage of forming the ingot, its outer skin 25 is quite tender and cracks are likely to form unless a perfectly free contraction of the ingot is possible without the sticking or adhering of the outer surface of the ingot to the inner surface of the mold. These cracks 30 in the surface of the ingot, as is well known, result in seams and surface defects that are produced when rolling the ingot.

It has been customary heretofore to coat 35 the inner surface of the mold to insulate the inner mold surface and to prevent adhesion of the ingot to said surface during the cooling process. To this end, various washes, consisting of mixtures of water with clay, 40 ganister, lime, or graphite, in certain proportions to give the proper fluid consistency, have been used. These washes have been applied in various ways, as for example, by spraying, by means of brushes or swabs, and by splashing,—the end and aim in each case, 45 being to cover as much of the inside surface of the mold as possible. None of the above methods, however, have been capable of depositing the insulating, non-adherent wash 50 in a uniform layer or film upon the inside 55 surface of the mold.

The object of my improved process and apparatus is to apply an insulating wash of the kind described, in a uniform, even, smooth layer or film, completely covering the entire inner surface of the mold, and 60 filling in and smoothing over all inequalities and depressions therein.

In carrying out my process, I provide a wash consisting of water and of clay, ganister, lime, or graphite, in the necessary 65 proportions to produce a mixture of such fluid consistency that it will stick or adhere to the surface of the mold when applied thereto. This mixture is placed in a tank or other suitable reservoir, and the mold 70 is partly or wholly dipped into, or submerged in the fluid mixture, so as to bring all of the inner surface of the mold into contact with the mixture or wash.

The mold is then withdrawn from the 75 fluid mixture and the outside surface of the mold is washed or cleaned by sprays of water or otherwise, to remove the insulating wash or mixture from the outer surface of the mold. The mold is then in readiness 80 for use in pouring the molten metal to form the ingot.

The accompanying drawings illustrate my improved apparatus and will more clearly and fully demonstrate my improved process. 85

In the drawings:

Figure 1 is a diagrammatic view, representing in vertical elevation and partially in vertical section, an apparatus for carrying out the process.

Fig. 2 is a view showing the dipping tank in vertical section, in a plane at right angles to that of Fig. 1, with the mold car placed adjacent thereto.

Fig. 3 is a top plan view of the dipping tank.

Referring now to that embodiment of my improved apparatus for carrying out my process:

10—10 indicate the upright beams of a 100 traveling crane structure; 11—11, the upright posts; 12—12, I-beam stringers, and 13—13, the rails supported thereon, and providing tracks for the wheels 14—14 of a traveling crane 15. The upright beams 105 10—10 are connected together at the top by suitable tie members 16, and the I-beams 12 are braced from said upright members by means of plates 17—17; 18 indicates a transverse shaft mounted on the traveling crane 110

15 and adapted through suitable gearing 19-19 to drive the wheels 14-14 along the tracks 13-13; 20 indicates the motor for driving the shaft, and 21, the operator's cab 5 in which is provided suitable mechanism for controlling the motor. 22 indicates a transversely moving carriage mounted on rails 23 on the top of the traveling crane 15; a differential drum 24 is mounted on this carriage, and is driven by gearing 25, actuated in a familiar manner by a motor 26 mounted on the carriage, and arranged for control by the operator in the cab 21.

27 indicates an open vessel or tank set in 15 the ground or floor 28, upon which the traveling crane structure is erected. This tank consists, as shown, of a substantially rectangular box made of concrete or other suitable material, and preferably provided with 20 a metallic sheet lining 29. This tank, as shown, projects above the floor or ground level 28. A trackway 30 is arranged alongside the tank 27 for a mold car 31. The tank 27 constitutes the dipping tank and 25 contains the mixture of insulating wash or fluid, consisting of water and of one of the several substances, clay, ganister, lime or graphite, as heretofore described.

The dipping tank is provided with means 30 for agitating the fluid mixture contained therein. As shown, this means consists of an air blast pipe 32 which is located at one side of the tank and which depends into the tank to a point near the bottom thereof. 35 There is also provided means for heating the dipping mixture, which, as shown, consists of a steam pipe 33 leading from any convenient source of steam supply (not shown) and depending into the tank.

40 About the top of the dipping tank, there is placed a perforated pipe 34 built in the form of a hollow rectangle, with the perforations directed toward the interior of the tank, and connected to a supply pipe 35. Said pipe has a hand valve 36 adapted to 45 admit water under pressure into the pipe 34, from which it will be discharged through the perforations therein into the space defined by the four upright walls of the tank.

50 In the bottom of the tank is placed a basket 37 which is preferably in the form of a shallow, rectangular, open box having a perforated bottom wall 38. This basket is provided with chains 39 connected to its 55 four corners,—there being one chain at each end of the basket. Said chains are normally looped upon hooks 40 fixed in the end walls of the tank 27 near its top. These chains may be engaged by the grapple of the 60 traveling crane 15 to withdraw the basket from the tank, as will be presently described.

45 indicates the ingot molds. Said molds (one or more at a time,—two, as shown) are dipped in the fluid mixture in the tank by 65 means of a grapple 46 attached to the blocks

47 connected in the usual manner by means of ropes or chains 48, to the differential drum 24 of the traveling crane. The grapple is operated by the usual trip rope 49 in such a manner as to connect with or to be detached from the usual ears 45<sup>a</sup> on the molds 45.

In carrying out the improved process by means of the novel apparatus hereinbefore described, the dipping tank is filled with 75 one of the fluid insulating mixtures heretofore described. Steam is admitted through the pipe 33 in order to heat the mixture to a point somewhat below that of boiling water. At the same time, in order to maintain a thorough mixture of the wash, in which the solid material is merely suspended and not dissolved, air under pressure is admitted through the air pipe, and this air, escaping under the surface of the fluid in the tank, will agitate the mixture, maintain the solid material in suspension and produce and maintain a constant, uniform mixture.

A number of molds 45 are brought on the mold car 31 into a position adjacent to the tank 27. The traveling crane and the carriage 22 thereon, are brought in a familiar manner above the molds on the mold car, and the block and grapple 47-46, are operated to lift the molds from the mold car and to lower them into the tank 27 until they are completely immersed in the insulating fluid mixture therein. The molds are allowed to remain therein until a film or coating of the insulating mixture has adhered to the surface of the molds. The differential drum of the crane is then operated to raise the mold from the dipping tank. As it is raised, the valve 36 is opened to supply water through the pipe 34, and this water is discharged through the perforations of said pipe against the mold, so as to clean and remove the wash or insulating mixture from its outer surface. The mixture, after it is washed off the outer surface of the mold, drips back into the tank together with the wash water. The dipped molds are then returned to the mold car, and another mold or set of molds is brought above the tank and dipped into it, the process being continued as before. After all the molds have been treated in this way by the dipping process, they are taken away and the molten steel is poured into them in the usual manner.

The fluid mixture in the dipping tank is kept at a temperature between 100° and 200° F. The advantage of maintaining the fluid mixture at this temperature, is that cold molds will be warmed up and raised to a temperature above that of the atmosphere during the dipping process, so that they will be in a more desirable condition as to temperature to receive the molten steel poured into them. Again, by maintaining the tem- 130

perature of the dipping mixture at the degree described, the chilling of hot molds, when dipped into the mixture, is prevented.

The spray water pipe 34 not only acts to 5 clean the outside surface of the mold and remove the insulating mixture therefrom, but it also, being cold and dripping into the dipping tank, keeps down the temperature of the dipping mixture below the boiling 10 point of water, when the temperature of the mold that is being treated exceeds that temperature. The addition of water, in this washing process, to the fluid mixture in the dipping tank, is compensated for by the 15 evaporation that takes place, due to the temperature of the dipping mixture.

By the dipping process herein described, the interior surface of the mold is provided with a smooth, uniform layer of insulating 20 material, and this layer or coating is applied to every part of the said interior surface. Said uniform coating not only protects the mold, and prolongs its life, but it obviates surface flaws in the ingot and permits free 25 stripping of the steel from the inner surface of the mold as the ingot contracts. In addition, when the steel is poured, the small particles of molten metal that are splashed or thrown up against the mold surface as 30 the molten steel rises therein, do not stick to the surface of the mold, but drop back into the molten mass.

Any sediment or particles of foreign substance that fall into the dipping tank, will 35 collect in the basket 37, which may be withdrawn at intervals to remove the same.

In describing the process, I have illustrated apparatus by which the mold is completely submerged in the fluid mixture contained 40 in the dipping tank. It will be understood, of course, that complete submersion is not necessary, it being simply required to immerse the mold to such an extent that the fluid, insulating mixture will 45 be brought into contact with the entire interior surface of the mold, or with so much of said surface as will be brought into contact with the molten metal, when the ingot is poured.

50 I claim as my invention:

1. The process of applying a uniform layer of insulating material upon the inner surface of an ingot mold having a vertically elongated ingot chamber, which consists in 55 dipping the mold into a fluid mixture of the insulating material so as to completely immerse the interior surface of the mold therein, and in then removing the coating of insulating material collected on the outer 60 surface of the mold during the dipping process.

2. The process of applying a uniform layer of insulating material upon the inner surface of an ingot mold having a vertically 65 elongated, tubular ingot chamber, which

consists in dipping the mold when in a substantially erect position into a fluid mixture of insulating material so as to completely immerse the interior surface of the mold therein, said mixture being maintained 70 at a temperature of 100° F. or more.

3. The process of applying a uniform layer of insulating material upon the inner surface of an ingot mold having a vertically disposed ingot chamber, which consists in 75 dipping the mold when in a substantially erect position into a fluid mixture of the insulating material so as to completely immerse the interior surface of the mold therein, and in then removing the coating of the 80 material collected on the outer surface of the mold during the dipping process, as the mold is withdrawn from said mixture.

4. The process of applying a uniform layer of insulating material upon the inner 85 surface of an ingot mold having a vertically disposed ingot chamber, which consists in dipping the mold when in a substantially erect position in a fluid mixture of the insulating material, which is maintained at a 90 temperature of from 100° to 200° F., the mold being dipped into the fluid mixture of the insulating material so as to completely immerse its interior surface, and in washing the insulating material collected on the 95 outer surface of the mold from said outer surface, as the mold is withdrawn from the mixture.

5. The process of applying a uniform layer of insulating material upon the inner 100 surface of an ingot mold having a vertically disposed ingot chamber, which consists in dipping the mold when in a substantially erect position into a fluid mixture of the insulating material so as to completely immerse the interior surface of the mold therein, in agitating the fluid mixture during 105 the dipping process, in heating the mixture to a temperature substantially between 100° and 200° F., and in washing therefrom 110 the insulating material collected on the outer surface of the mold in the dipping process, as the mold is withdrawn from said mixture.

6. The process of applying a uniform 115 layer of insulating material upon the inner surface of an ingot mold having a vertically disposed ingot chamber, which consists in dipping the mold when in a substantially erect position into a fluid mixture of the insulating material, in agitating said mixture during the dipping process, in heating said mixture to a temperature between 100° 120 and 200° F., and in discharging a spray of water against the outer surface of said mold 125 to remove the insulating material collected thereon.

7. The process of applying a uniform layer of insulating material upon the inner 130 surface of an ingot mold having a vertically

disposed ingot chamber, which consists in immersing the mold when in a substantially erect position in a tank containing a fluid mixture of insulating material so as to completely cover the interior surface of said mold, in agitating the mixture in said tank, in heating said mixture to a temperature between 100° and 200° F., and in washing the outer surface of said mold as it is withdrawn from said tank, with cold water, and allowing said water, together with the

insulating material washed from the outer surface of the mold to drop back into said tank.

In testimony that I claim the foregoing <sup>15</sup> as my invention I affix my signature in the presence of two witnesses, this 11th day of December, A. D. 1916.

GEORGE FRANCIS DOWNS.

Witnesses:

JULIA G. WUNSCH,  
WALTER J. BRYAN.